

## UNITED STATES PATENT OFFICE

2,078,861

## MANUFACTURE OF AZO DYESTUFFS

Robert Lantz, Paris, France, assignor to Societe Anonyme des Matieres Colorantes & Produits Chimiques de Saint-Denis, Paris, France, a company of France

No Drawing. Application December 16, 1935,  
Serial No. 54,789. In France December 22,  
1934

## 14 Claims. (Cl. 8—5)

Mixtures of aryl anti-diazosulphonates or aryl hydrazine-sulphonates with azo coupling components are stable under ordinary conditions and their solutions do not undergo spontaneous coupling. It is known that these mixtures can be caused to undergo coupling by the action of light (see particularly French Patent No. 760,784) or in the case of certain particular diazosulphonates applied to fibrous material by impregnation, by the action of a steaming operation (see German Patents Nos. 560,797, 563,061, 560,798 and 578,648).

The present invention relates to the production of azo-dyestuffs in substance or on a fibre which also makes use of mixtures of coupling components with aromatic anti-diazosulphonates or hydrazine-sulphonates i. e. with aromatic compounds in which a sulphonic group is connected to an aryl group by a dinitrogen group. In accordance with the present invention the mixture is caused to undergo coupling by subjecting it to the action of an energetic oxidizing agent and then, if required, to the action of an alkaline agent.

The invention is of special importance in its application to the production of insoluble azo-dyestuffs on textile fibres. For this purpose there are used diazosulphonates or hydrazine-sulphonates prepared from aromatic amines which are free from groups which impart solubility, such as COOH or SO<sub>3</sub>H and coupling components which are likewise free from these groups. Since the coupling components generally contain hydroxyl groups which render them soluble in alkaline media, an alkaline solution of the mixture can be used for the impregnation of the fibre. This impregnation may extend throughout the material or may be only local so that after development there will be produced a dyeing or a print respectively. The solutions may, of course, contain all the known ingredients which are used in dyeing and printing and especially in the production of insoluble azo-dyestuffs on fibrous materials by means of a single mixture containing the two coupling substances (rapid solid dyestuffs, rapidogens, dyestuffs obtained with the aid of nitrosamines).

The oxidation may occur in a gaseous or liquid medium. Among the oxidizing agents which are useful for carrying out the invention there may be named chlorine and bromine in the form of a solution or in gaseous state, hypochlorites and bromates in the presence of an acid, nitrous acid, lead peroxide in an acid medium and so on. In the production of the dyestuffs on fibrous material the oxidation may occur in a liquid medium or by exposure to an atmosphere containing a gaseous oxidizing agent.

The course of the process is quite unexpected for it was to be supposed that the oxidizing agent would first attack the azo-coupling components which are readily oxidized and would thus render coupling impracticable.

The dyestuff may be formed actually in the course of the oxidation or it may be formed in a subsequent treatment, generally an alkaline treatment which itself may be conducted in a liquid or gaseous medium. In order to prepare the dyestuff in a single stage the oxidation may be conducted at a temperature higher than ordinary temperature; thus the dyestuffs may be formed on the fibre by treating the fibre impregnated with the selected mixture with a halogen in presence of hot water or steam.

The diazosulphonates or hydrazine-sulphonates which are best suited for carrying out the invention are those which are prepared from feebly basic aromatic amines containing in the molecule a negative substituent such as a nitro-group or halogen and so on.

For the production of azo-dyestuffs on fibrous material in accordance with the invention there are advantageously used azo-components of the type hitherto used industrially for a like purpose, such as the arylides of organic acids capable of coupling, particularly the arylides of  $\beta$ -oxynaphthoic acid, of 2-hydroxyanthracene-3-carboxylic acid, of oxycarbazole and oxynaphthocarbazole carboxylic acids, of carboxylic acids having a coupling position in a methylene group which may or may not form part of a ring, such as acyl acetic acids, aroyl acetic acids and so on.

Insoluble azo-dyestuffs can be produced in accordance with the present invention on the various animal and vegetable fibres and on artificial fibres of regenerated cellulose, cellulose ethers or cellulose esters.

The following examples illustrate the invention, the parts in Examples 6 and 7 being by weight:

## Example 1

A cotton fabric is printed with the following mixture:

|                                                                  | Grams  |
|------------------------------------------------------------------|--------|
| Sodium 2-methyl-5-chlorobenzene diazo-sulphonate                 | 20     |
| 1 - (2' - hydroxy - 3' - naphthoyl) - amino - 2 - methyl-benzene | 20 50  |
| Alcohol                                                          | 20     |
| Caustic soda solution of 40° Bé.                                 | 20     |
| Glycerine                                                        | 50     |
| Starch tragacanth thickening                                     | 500    |
| Water                                                            | 390 55 |

After the material has been dried it is treated for 3 seconds in an apparatus containing steam and chlorine at 100° C. in order to develop the dyeing. Then the fabric is washed and treated in a boiling bath containing soap and sodium carbonate. There are obtained beautiful red prints.

Like prints are obtained by printing the same mixture on fabrics of artificial silk of viscose or acetyl cellulose, or natural silk or wool.

By replacing the two components in the foregoing example by other diazosulphonates and coupling components there are obtained the 15 shades indicated in the following table:

|    | Diazosulphonate                                                                                                                                                                                      | Coupling component: (2'-hydroxy-3'-naphthoyl)-                       | Shade                                       |    |
|----|------------------------------------------------------------------------------------------------------------------------------------------------------------------------------------------------------|----------------------------------------------------------------------|---------------------------------------------|----|
| 5  | Sodium 2-nitrobenzene-diazosulphonate.<br>Do.....                                                                                                                                                    | 1-amino-2-methylbenzene.<br>1-amino-2-methoxybenzene.                | Yellowish red.<br>Red orange.               | 5  |
| 10 | Sodium 2-methoxy-4-nitrobenzene-diazosulphonate.<br>Do.....                                                                                                                                          | 1-(2'-hydroxyanthra-<br>cene-3'-carboxylamino)-2-methylben-<br>zene. | Bluish black<br>violet.                     | 10 |
| 15 | Sodium 2-nitro-4-methylbenzene-diazosulphonate.<br>Sodium 3-nitro-6-methylbenzene-diazosulphonate.<br>Sodium 3-chloro-6-methylbenzene-diazosulphonate.<br>Sodium 2,5-dichlorobenzenediazosulphonate. | 1-(2'-hydroxyanthra-<br>cene-3'-carboxylamino)-2-methylben-<br>zene. | Brown red.<br>Dull violet.<br>Do.<br>Brown. | 15 |
| 20 | Sodium 2-nitro-4-methylbenzene-diazosulphonate.<br>Do.....                                                                                                                                           | 1-(2'-hydroxyanthra-<br>cene-3'-carboxylamino)-2-methylben-<br>zene. | Dull violet.<br>Brown red.                  | 20 |
| 25 | Do.....                                                                                                                                                                                              | 1-(2'-hydroxyanthra-<br>cene-3'-carboxylamino)-2-methylben-<br>zene. | Yellow brown.<br>Do.                        | 25 |
| 30 | Do.....                                                                                                                                                                                              | 1-(2'-hydroxyanthra-<br>cene-3'-carboxylamino)-2-methylben-<br>zene. | Yellow brown.                               | 30 |
| 35 | Sodium 2-nitro-4-methylbenzene-diazosulphonate.<br>Do.....                                                                                                                                           | 1-(2'-hydroxyanthra-<br>cene-3'-carboxylamino)-2-methylben-<br>zene. | Brown.<br>Do.                               | 35 |
| 40 | Sodium 2-nitro-4-methylbenzene-diazosulphonate.<br>Do.....                                                                                                                                           | 1-(2'-hydroxyanthra-<br>cene-3'-carboxylamino)-2-methylben-<br>zene. | Yellowish grey.                             | 40 |
| 45 | Sodium 3-nitro-6-methylbenzene-diazosulphonate.<br>Do.....                                                                                                                                           | 1-(2'-hydroxyanthra-<br>cene-3'-carboxylamino)-2-methylben-<br>zene. | Reddish black<br>violet.                    | 45 |
| 50 | Sodium 3-chloro-6-methylbenzene-diazosulphonate.<br>Do.....                                                                                                                                          | 1-(2'-hydroxyanthra-<br>cene-3'-carboxylamino)-2-methylben-<br>zene. | Yellow.                                     | 50 |
| 55 | Sodium 2,5-dichlorobenzenediazosulphonate.<br>Do.....                                                                                                                                                | 1-(2'-hydroxyanthra-<br>cene-3'-carboxylamino)-2-methylben-<br>zene. | Reddish yellow.                             | 55 |
| 60 | Sodium 2-nitrobenzene-diazosulphonate.<br>Aminobenzene.....                                                                                                                                          | 1-(2'-hydroxyanthra-<br>cene-3'-carboxylamino)-2-methylben-<br>zene. | Do.                                         | 60 |
| 65 | Do.....                                                                                                                                                                                              | 1-(2'-hydroxyanthra-<br>cene-3'-carboxylamino)-2-methylben-<br>zene. | Do.                                         | 65 |
| 70 | Sodium 3-nitro-6-methoxybenzene-diazosulphonate.<br>Do.....                                                                                                                                          | 1-(2'-hydroxyanthra-<br>cene-3'-carboxylamino)-2-methylben-<br>zene. | Do.                                         | 70 |
| 75 | Sodium 2-nitrobenzene-diazosulphonate.<br>Do.....                                                                                                                                                    | 1-(2'-hydroxyanthra-<br>cene-3'-carboxylamino)-2-methylben-<br>zene. | Do.                                         | 75 |

## Example 2

A cotton fabric is printed with the following mixture:

|                                                   | Grams |
|---------------------------------------------------|-------|
| Sodium 2-nitrobenzene-diazosulphonate             | 15    |
| 1-(2'-hydroxy-3'-naphthoyl)-amino-2-methylbenzene | 15    |
| Caustic soda solution of 40° Bé                   | 14    |
| Starch tragacanth thickening                      | 500   |
| Water                                             | 412   |

After the fabric has been dried it is passed, during several seconds, through an aqueous solution of chlorine having a temperature of 70° C. yellowish-scarlet prints are obtained.

In like manner there are obtained with sodium 2-nitro-4-methylbenzene diazosulphonate and 1-2'-hydroxy-3'-naphthoyl)-amino-2-methoxybenzene bluish-red prints. Development may be conducted in an analogous manner with bromine water.

By using in the printing preparation sodium 2:5-dichlorobenzene-diazosulphonate and 1-(2'-hydroxy-3'-naphthoyl)-amino-2-methylbenzene and developing the dyeing by means of a boiling 5 salt solution of 20 per cent strength through which chlorine is passed there are obtained yellowish-scarlet prints.

*Example 3*

10 If in Example 1 the sodium 5-chloro-2-methylbenzene-diazosulphonate is replaced by the corresponding quantity of 5-chloro-2-methylbenzene hydrazine sulphonic acid and the operation is 15 conducted otherwise as therein prescribed there are obtained prints of the same shade.

*Example 4*

Printing is conducted as in Example 1 but with 20 the use of sodium 2-methoxy-4-chlorobenzene diazosulphonate and 1-(2'-hydroxy-3'-naphthoyl)-amino-2-methoxybenzene. The dyeing is developed by passing the moist material during several seconds first through an atmosphere of 25 chlorine and then through an atmosphere of ammonia or through a solution of sodium carbonate. Red prints are obtained.

*Example 5*

30 A cotton fabric is impregnated with the following preparation:—

|                                                                | Grams |
|----------------------------------------------------------------|-------|
| Sodium 2-methyl-5-chlorobenzene diazosulphonate                | 20    |
| 1 - (2' - hydroxy- 3' - naphthoyl) - amino - 2 - methylbenzene | 20    |
| Alcohol                                                        | 20    |
| Caustic soda solution of 40° Bé.                               | 20    |
| Glycerine                                                      | 50    |
| 40 Tragacanth mucilage of 6 per cent strength                  | 100   |
| Water                                                          | 770   |

The material is dried and treated as described in Example 1 to develop the dyeing. A beautiful 45 red dyeing is thus obtained.

*Example 6*

A current of chlorine is passed slowly through 50 a cold solution prepared from 10 parts of sodium 2-methyl-5-chlorobenzene diazosulphonate, 10 parts of 1-(2'-hydroxy-3'-naphthoyl)-amino-2-methylbenzene, 10 parts of alcohol, 10 parts of caustic soda solution of 40° Bé. and 960 parts of 55 water. There is at once formed a red precipitate which gradually increases in bulk. When no further precipitation occurs the current of chlorine is interrupted and the dyestuff is filtered and dried.

*Example 7*

A solution is prepared by dissolving 1 part of sodium 2-hydroxy-naphthalene-6-sulphonate, 1 part of sodium 2-methyl-5-chlorobenzene diazo- 65 sulphonate, 0.8 part of sodium bicarbonate and 2 parts of sodium chloride in 100 parts of water and a current of chlorine is passed through the solution. There is at once precipitated an orange-red dyestuff which is isolated by saturating the 70 solution with salt and filtering. The dyestuff is identical with that obtained by the direct action of 2-methyl-5-chlorobenzene diazonium chloride on sodium 2-hydroxynaphthalene-6-sulphonate. It dyes wool an orange shade.

75 The diazosulphonates referred to herein may

be prepared by any suitable process and particularly in the manner indicated in French Patent No. 760,784.

What I claim is:

1. A method of manufacturing azo-dyestuffs, 5 which comprises, treating with an oxidizing agent a mixture of an azo-coupling component and a salt of a sulphonic derivative of an aryl compound in which the sulphonic group is connected to the aryl nucleus through a dinitrogen 10 group.

2. A method of manufacturing azo-dyestuffs, 15 which comprises, treating with an oxidizing agent a mixture of an azo-coupling component and a salt of an aryl anti-diazo sulphonic acid. 15

3. A method of manufacturing azo-dyestuffs, 20 which comprises, treating with an oxidizing agent a mixture of an azo-coupling component and a salt of an aryl hydrazine sulphonic acid.

4. A method of manufacturing azo-dyestuffs, 25 which comprises, treating a mixture of an azo-coupling component and a salt of a sulphonic derivative of an aryl compound, in which the sulphonic group is connected to the aryl nucleus through a dinitrogen group, with an oxidizing 25 agent and subsequently with an alkaline agent.

5. A method according to claim 1 in which said salt contains in the nucleus an electro-negative group.

6. A method according to claim 1 in which 30 said salt contains in the nucleus a halogen group.

7. A method according to claim 1 in which said salt contains in the nucleus a nitro-group.

8. A method according to claim 1 in which 35 said coupling component is an arylide of an organic acid capable of coupling.

9. A method of producing insoluble dyestuffs on fibrous material, which comprises, impregnating said material simultaneously with an oxidizing agent and a mixture of an azo-coupling component and a salt of a sulphonic derivative of an aryl compound in which the sulphonic group is connected to the aryl nucleus through a dinitrogen group, neither of these components including a solubilizing group apart from said sulphonic 45 group, and treating said impregnated fibrous material with a halogen in the presence of water.

10. A method according to claim 9 in which 50 said water is in the form of steam.

11. A method for producing water insoluble 50 azo-dyestuffs on a fibrous material, which comprises applying to said fibrous material a mixture including an azo-coupling component and a salt of a sulphonic derivative of an aryl compound in which the sulphonic group is connected to the 55 aryl nucleus through a dinitrogen group, neither of said azo-coupling component and said salt including a water solubilizing group apart from said sulphonic group, and subjecting said mixture on the fibrous material to the action of an oxidizing agent.

12. The method of claim 11, further comprising subjecting said mixture on the fibrous material to a subsequent treatment with an alkaline 65 agent.

13. A method of dyeing a fibrous material which comprises applying to said fibrous material an alkaline mixture including an azo-coupling component and a salt of a sulphonic derivative of an aryl compound containing at least one 70 hydroxyl group, in which the sulphonic group is connected to the aryl nucleus through a dinitrogen group, neither of said azo-coupling component and said salt including a water solubilizing group apart from said sulphonic group, and sub- 75

jecting said mixture on the fibrous material to the action of an oxidizing agent.

14. The method of developing a normally stable mixture of an azo-coupling component and a salt of a sulphonic derivative of an aryl compound in which the sulphonic group is connected to the

aryl nucleus through a dinitrogen group, so as to produce an azo-dyestuff, which method consists in exposing said mixture to an energetically oxidizing medium at a temperature higher than ordinary temperature, for a short time.

ROBERT LANTZ.